

## UNITED STATES PATENT OFFICE.

BERTRAND S. SUMMERS, OF PORT HURON, MICHIGAN.

PROCESS FOR ELECTRODEPOSITING LEAD UPON IRON.

No Drawing.

Application filed February 23, 1923. Serial No. 620,825.

*To all whom it may concern:*

Be it known that I, BERTRAND S. SUMMERS, a citizen of the United States, residing at Port Huron, in the county of St. 5 Clair and State of Michigan, have invented certain new and useful Improvements in Processes for Electrodepositing Lead Upon Iron, of which the following is a specification.

10 It has long been a matter of common practice to line iron pipes and to cover other articles of iron with a thin lead coating in order to protect them from rust, particularly where they are exposed to moisture. This 15 coating is ordinarily applied by electro deposition from an aqueous bath or solution. It has been found difficult or impossible heretofore to produce in this manner a dense homogeneous coating of the metal which is 20 uniformly adherent and of good appearance, particularly where a sufficient current density is employed to meet the demand of rapid operation. While my invention is primarily designed for plating iron, it is obvious 25 that other metals may be used where a suitable protective coating is desired.

By the invention which forms the subject matter of this application I have been able to rapidly form a dense coating of 30 the required thickness which is tenaciously adherent throughout and substantially free from discoloration. In my improved process for depositing lead on iron I employ a solution of lead acetate and anodes of aluminum. Preferably and in the specific example of the invention herein given, the acetate of lead is dissolved in a bath of acetate of aluminum containing also acetate of lime formed by dissolving alum in acetate of 35 lime. I prefer to use the crude form of the acetate of lime on account of the impurities found therein which are of organic nature due to the source of the acetate of lime and form a suitable colloid which tends to 40 prevent the formation of sponge during the plating. The acetate of lime is preferably used in excess for this reason. With the electrolytic bath formed in this way the metal forming the cathode receives a much 45 more uniform, denser coat free from stain and a much higher current density can be used in the operation which naturally cuts down the required time. The explanation of the superior results is not definitely known but the ions of aluminum undoubt- 50 edly have some effect in aiding the deposi-

tion of the lead upon the cathode and alloying with the same and the electro-chemical equivalent of aluminum is very much smaller than lead, the deposition naturally consists chiefly of lead. The deposition formed is very resistant to acids and forms an admirable protective coating.

It has been found difficult to plate lead from its salts and in the cases where this has been done, it is usually necessary to keep the current density rather low to avoid forming trees or sponges. I have discovered that if a compound anode is used, that is, lead and aluminum, a coating is plated on 65 the cathode which is very dense, resistant to acids, and which may be plated with a high current density.

As a specific illustration of the practice of my improved process I give the following: 500 pounds of alum and 1000 pounds of acetate of lime were dissolved in about 2000 gallons of water. After the deposition ceased the clear liquid consisting of a solution of acetate of aluminum and a proportion of acetate of lime with, doubtless, an amount of organic or colloidal matter was decanted and 500 pounds of lead acetate dissolved therein. Iron pipe which was the article to be coated, after being pickled and cleaned in the usual manner, was connected as the cathode and aluminum anodes were employed, the anodes and cathodes being connected up to a suitable source of direct current. At the outset the current employed 75 was small, about two amperes or less per square foot of the cathode surface being employed, and as the initial film formed the current density was gradually increased until it amounted to ten amperes per square 80 foot. The plating operation was continued with the greater current density until a plating of the desired thickness had been deposited. The temperature employed was very slightly above the atmospheric temperature at the time, though it might have been slightly greater or less without materially affecting the result. After the desired thickness had been deposited, the pipe was removed from the bath and thoroughly 85 washed to cleanse it of the electrolyte.

The resultant coating was an alloy of lead containing a small percentage of aluminum and was dense, uniform in color and thickness, and closely adherent to the base metal throughout and could be peeled therefrom only with the greatest difficulty.

I claim:

1. A process of electro-plating lead on iron which consists in forming a solution of lead, immersing the iron to be treated therein, immersing aluminum anodes therein and connecting the anodes and the iron cathodes with a suitable source of direct current.
2. A process of plating lead on iron which consists in forming an electrolyte containing lead in solution, immersing the articles to be coated in the electrolyte, connecting them as the cathode and an anode immersed in the electrolyte to a source of direct current, passing a current of low cathode density from the anodes through the electrolyte to the cathodes and gradually increasing the current density.
3. A process of electro-plating iron with lead which consists in forming an electrolyte containing acetate of lead, aluminum acetate and calcium acetate, immersing the iron articles to be treated as a cathode in the electrolyte, immersing an aluminum anode in the electrolyte and passing a plating current from said anode to the cathode.
4. A process of electro-plating lead on iron which consists in dissolving an aluminum salt in a solution of acetate of lime, dissolving lead acetate in the solution so formed, immersing the iron articles to be coated and aluminum anodes in the electro-
5. A process of electro-plating lead on iron which consists in dissolving alum in a solution containing an excess of acetate of lime thereby forming a solution of acetate of aluminum containing acetate of lime, dissolving lead acetate in said solution to form an electrolyte, immersing aluminum anodes and the iron to be plated in the electrolyte so formed, and passing a plating current from the anode to the cathode.
6. A process of electro-plating lead on a metal base which consists in forming a solution of lead, immersing the metal to be plated therein, and immersing in the plating bath aluminum and lead anodes and connecting the anodes and the cathode formed by the metal to be plated with a substantial source of a direct current.
7. A process of electro-plating lead on iron which consists in electro-depositing lead on iron in a bath containing a soluble salt of lead and a third metal in a form in which it will not react with the lead salt.
8. A process of electro-plating lead on iron which consists in electro-depositing the lead from a bath containing a soluble salt of lead and aluminum in a form in which it will not react with the lead salt.

BERTRAND S. SUMMERS.